

A. PIETZSCH & G. ADOLPH.  
ELECTRODE FOR PREVENTING CATHODIC REDUCTION.  
APPLICATION FILED OCT. 3, 1912.

1,083,132.

Patented Dec. 30, 1913.



Witnesses.  
E. Knobell.  
J. W. Price.

Albert Piltzsch & Inventors  
Gustav Adolph  
by Wilkinson, Giese  
& Mackay  
Their Attorneys

# UNITED STATES PATENT OFFICE.

ALBERT PIETZSCH AND GUSTAV ADOLPH, OF MUNICH, GERMANY.

## ELECTRODE FOR PREVENTING CATHODIC REDUCTION.

1,083,132.

Specification of Letters Patent.

Patented Dec. 30, 1913.

Application filed October 3, 1912. Serial No. 723,788.

To all whom it may concern:

Be it known that we, ALBERT PIETZSCH, engineer, a subject of the King of Saxony, and resident of Munich, Germany, and Dr.

5 GUSTAV ADOLPH, chemist, a subject of the King of Prussia, and resident of Munich, Germany, have invented a new and useful Arrangement of Electrodes for Preventing Cathodic Reduction, of which the following is a full, clear, and exact specification.

10 There are many cases in which it is necessary to prevent reducing action of the cathode in an electrolytic cell. In such cases it has been usual hitherto either to separate 15 the two electrodes by a diaphragm or to make additions to the electrolyte which form a diaphragm immediately on the surface of the cathode, for example a diaphragm of chromium oxid, of potassium resinate and 20 the like. While the first method has the disadvantage of being expensive and of greatly increasing the resistance of the bath, the latter method can only be used for preventing reduction in alkaline or neutral solutions. 25 Moreover the additions to the electrolyte produce at least to a certain extent a disturbance of its purity and coloration.

Now it is possible to prevent cathodic reduction in a very simple manner if the 30 cathode body is wrapped up closely with a thread made from porous non-conducting and chemically inert fibers in such a way that the bubbles of hydrogen forming upon the cathode escape between the separate 35 turns of the thread. This arrangement has the surprising effect that the circulation of the electrolyte immediately on the surface of the cathode is so effectively prevented that the main bulk of the electrolyte practically 40 does not come into contact with the surface of the cathode at all. The arrangement has the advantage of great cheapness and forms a very simple and stable construction; it does not give rise to any impurity of electrolyte 45 and even has frequently a special advantage inasmuch as the electrolyte is well stirred by the passage of the hydrogen bubbles through the anode space. It may be used both in alkaline and also, which was hitherto not possible, in acid solutions, for 50 example in the production of persulfates,

hypochlorite lyes, chlorates and in short of all reducible substances which are obtained electrically whether the solutions be acid or alkaline.

55

Example I: According to the annexed drawing a rod 1 of carbon of 20 mm. diameter is closely wound around with asbestos string 2 of 3 mm. diameter, there being about 330 turns per meter length of rod. 60 The use of such a rod as cathode enables ammonium persulfate solution of up to 300 gr. per liter to be produced from strong acid ammonium sulfate solution, the reduction not exceeding 5% at the end of the electrolysis.

65 Example II: A rod made in the same way can be used as cathode in an electrolyzer for bleaching solution; not more than 3% reduction has to be reckoned with when the 70 bleaching solution has attained a strength of 25 gr. of active chlorin per liter.

What we claim is:

1. An electrode for preventing cathodic reduction, constituted by a cathode body 75 closely wrapped up with a porous thread of non-conducting fiber which cannot be chemically attacked, in such a way that as nearly as possible the whole surface of the cathode is covered in order that the bubbles 80 of hydrogen arising upon the cathode can escape between the separate turns of the thread into the anode space.

2. An electrode for preventing cathode reduction, constituted by cathode body 85 closely wound around with an asbestos string, in such a way that as nearly as possible the whole surface of the cathode is covered in order that the bubbles of hydrogen arising upon the cathode can escape between 90 the separate turns of the thread into the anode space.

In witness whereof we have hereunto signed our names this 20th day of September, 1912, in the presence of two subscribing 95 witnesses.

ALBERT PIETZSCH.  
DR. GUSTAV ADOLPH.

Witnesses:

RICHARD LEMP,  
MATHILDE K. HELEN.